

## UNITED STATES PATENT OFFICE

2,372,414

## METHOD OF PREPARING A LUBRICATING COMPOSITION

John F. Werder, Lakewood, Ohio, assignor, by direct and mesne assignments, to The Lubri-Zol Development Corporation, Cleveland, Ohio, a corporation of Delaware

No Drawing. Application January 17, 1933,  
Serial No. 652,199

1 Claim. (Cl. 252—58)

This invention relates to an improved form of lubricant and the process of making the same.

As is well known, the function of a lubricating medium is to maintain a film between surfaces which are subjected to frictional engagement. From a practical standpoint, the importance of lubrication is almost wholly confined to metal surfaces. The efficiency and life of any unit of machinery is almost wholly contingent upon the constant maintenance of an effective lubricating film.

With this in mind, there have been prior attempts to effect a combination between chlorine and lubricating oils because of the peculiar ability of chlorine to maintain surface tension and cohesion and prevent metal-to-metal contact under extreme conditions. I have found for example that carbon tetrachloride has very exceptional qualities as a cutting oil. Up to the present time, so far as I am aware, there has not been devised a method of combining chlorine with a lubricating oil so as to maintain a stable and permanent product.

The object of the present invention, therefore consists in producing a combination of chlorine and lubricating oil of such stable and permanent a character as to be employed in a practical manner.

The present invention is directed also to an improved process of effecting such a combination.

It is understood that the present invention may be applied to various forms of oils including animal, vegetable, and marine oils, as for instance the oils of lard, corn and sardine as well as those designated as mineral oils.

The degree of saturation and the chemical characteristics are of importance in effecting the combination. For instance, an unsaturated oil absorbs chlorine more readily than a saturated oil. Also, the affinity of chlorine to sulphur may be utilized. For example, I have discovered that a mineral oil with a substantial quantity of sulphur will readily hold chlorine. Also, a mineral oil, thoroughly refined to drive out the sulphur, will readily absorb chlorine after sulphur has been reintroduced by heat or some other method. According to the present invention, the oil may contain approximately from three per cent (3%) to five per cent (5%) of sulphur by weight.

The oil to be treated is placed in a tank, preferably glass-lined. With small laboratory samples, I have used metal or metal painted containers with success. In commercial quantities, the metal reacts in an uncertain way during the operation, but the commercial availability of glass-lined con-

tainers in all sizes eliminates the necessity of risking possible injurious results. In any event, chlorine is then released directly from a tank containing the same in liquid form and introduced into the body of the oil in any suitable manner so as to cause the chlorine to bubble therethrough. Hydrochloric acid is thrown off during the operation and is carried off by any suitable method. I have effectively employed a vacuum on top of the oil to accomplish this result when treating commercial quantities of oil.

Preferably this mixing of the chlorine with the oil will be effected while maintaining the same at approximately one hundred degrees Fahrenheit (100° F.). It is also preferable, though not necessary, to mix dry air with the chlorine, in approximately equal proportions, while it is being introduced into the oil.

It is to be understood that the process, as above outlined in a general way, may be employed in connection with any of the various oils above referred to, it being understood that the percentage composition and the degree of temperature may be varied according to circumstances.

Reference will now be had to one specific form of my present invention, this particular instance comprising the combination of chlorine and cottonseed oil. This particular combination comprises fifty gallons of cottonseed oil having a density corresponding to twenty-two degrees (22°) Baumé (lighter than water), and approximately one hundred (100) pounds of chlorine which is introduced into the oil in liquid form from the cask in which the same is contained.

The chlorine is introduced into the body of oil at the rate of approximately ten (10) to twenty (20) pounds per hour, depending upon the amount of vacuum and other controllable factors. At the conclusion of this part of the process, the combination of the chlorine and oil should have a gravity when at ordinary room temperature of approximately seven degrees (7°) Baumé, (above).

This combination of chlorine and oil is then heated to three hundred degrees Fahrenheit (300 F.) or above and free dry air is forced into the same through the same pipe or other means as employed for the introduction of the chlorine into the oil. This air is caused to bubble through the combined body of oil and chlorine for the purpose of driving the hydrochloric acid gas therefrom. As a result, the chlorine is retained in stable combination with the oil; and at this point of the process, this combination of oil and chlorine is found to have substantially the same

gravity when at ordinary room temperature as in

the former test above referred to, that is, approximately seven degrees (7°) Baumé, (above).

The compound thus produced constitutes a base which may then be added to any form or weight of lubricating oil as may be desired, the percentage composition being varied according to the character and grade of lubricant and also according to prevailing conditions of use to which the final form of lubricant is to be applied. The percentage of base added to the lubricating oil may thus vary in practically any proportions to the final body of lubricant which includes the base.

Actual comparative tests have demonstrated that the addition of my present improved form of compound or base to an oil, increases very decidedly its holding quality and likewise enables it to stand up under a greatly increased load before reaching the breaking point. In the following table there are given the results of such actual tests showing a comparison between a steam refined cylinder stock (plain oil) and the same oil to which my present compound was added in various proportions. The plain oil which was employed in these tests had a viscosity of one hundred and fifty (150) at two hundred and ten degrees Fahrenheit (210° F.).

| Character of lubricant   | Holding efficiency | Breaking point |
|--------------------------|--------------------|----------------|
| Plain oil                | Pounds             | Pounds         |
| Same oil with base (5%)  | 400                | 500            |
| Same oil with base (10%) | 1,200              | 1,400          |
| Same oil with base (15%) | 1,600              | 1,800          |
| Same oil with base (20%) | 12,000             | 2,000          |
|                          | 1,800              |                |

<sup>1</sup> Held full capacity of machine.

The results indicated in the above table show that with my compound or base there is a very positive increase in the holding efficiency of the lubricant and also an increase in the load to which the same can be subjected before reaching the breaking point.

The following table sets forth the results of actual tests made to determine the decrease in friction under heavy loads which is realized from my present improved compound or base. These tests were made with a two hundred pound (200 lb.) load and with the same character of oil as

in the other tests noted above, that is, with a plain oil (steam refined cylinder stock), having a viscosity of one hundred and fifty (150) at two hundred and ten degrees Fahrenheit (210° F.), first without my improved compound or base, and then with my compound or base added thereto.

| Lubricant            | Load   | Friction |
|----------------------|--------|----------|
| Plain oil            | Pounds | Watts    |
| Same with base (15%) | 200    | 400      |
|                      | 200    | 200      |

As will be seen from the above instance, the addition of my compound to the lubricant reduced the element of friction one-half.

Thus, from the tests noted in the above tables, it will be seen that the advantages obtained with my present compound or base in combination with lubricants are very marked, and the practical value of the same is thus very obvious.

Thus, I have devised a practical form of lubricating compound which is especially well adapted to maintain itself in the form of a film over the metal surfaces requiring lubrication, this particular adaptability and efficiency being afforded by the peculiar ability of the chlorine to hold the lubricating medium as a film over the metal surfaces, when these ingredients can be held together in a stable form of compound, as already explained.

This highly efficient form of lubricant with its obvious practical advantages is made possible by my improved process by which the chlorine and lubricant may be brought together and maintained in stable form. Thus, this particular lubricating compound is capable of being produced, handled, and employed in a practical and extremely efficient manner.

What I claim is:

A method for the production of a lubricant comprising chlorinating a petroleum fraction containing aliphatic compounds by treating such fraction with chlorine, treating said chlorinated materials with an alkali to remove unduly reactive and unstable constituents and to leave relatively stable chlorinated derivatives, and blending such relatively stable chlorinated derivatives with a lubricating medium.

JOHN F. WERDER.